

# UNITED STATES PATENT OFFICE.

ALFRED WILM, OF SCHLACHTENSEE, NEAR BERLIN, GERMANY.

## PROCESS OF IMPROVING ALLOYS.

1,083,903.

Specification of Letters Patent.

Patented Jan. 6, 1914.

No Drawing.

Application filed March 15, 1910. Serial No. 549,455.

To all whom it may concern:

Be it known that I, ALFRED WILM, a subject of the German Emperor, and residing at Schlachtensee, near Berlin, Germany, 5 have invented a certain new and useful Improved Process of Improving Alloys, of which the following is a specification.

My invention relates to a process for improving alloys such for example, as alloys 10 containing aluminum and magnesium.

The object of my invention is to impart to such alloys an increased strength, elasticity and hardness.

It has been customary heretofore to 15 heat to redness metals or alloys after they have been completely wrought or worked into the desired shape. The purpose of such heating to redness, however, has been to equalize or remove the strains which were 20 produced by the strain-producing operations, such for example, as cold rolling, drawing, pressing and similar operations, to which the material had been subjected in bringing it into the desired form. In such 25 prior methods, it has been usual to keep the temperature of such reheating as low as possible because it was found that such reheating to redness was accompanied by a loss of strength and hardness. It has also 30 been customary, when it was desired to avoid the loss of strength and hardness due to such heating to redness, to allow the formed material to age,—that is to say, to stand unused and unsubjected to any external 35 strains which might affect it,—until with lapse of time the internal strains gradually disappeared or at least were materially reduced. In other words, it has been old in the prior art to subject partly or completely 40 manufactured metallic objects to a relatively low temperature, or to store such objects cold for a time.

My process comprises subjecting an alloy material, comprising aluminum and magnesium, to a relatively high temperature of between about 420° C. and 580° C. and then, after it has been cooled either slowly or by chilling, storing said material for some time prior to use.

50 I have found that by this treatment a spontaneous improvement takes place in the material. Of course, it is to be understood that after this treatment has been given to the material it is not to be subjected to any 55 further heating in the course of manufac-

ture, because such subsequent heating if of any appreciable extent would destroy the advantageous result obtained by my process. Hence, with articles of such alloy which pass through any stage of manufacture requiring heating in bringing them into the desired form, it is necessary to await the completion of this heating stage of the manufacture before subjecting the object to my improved process.

60 By my improved process of treating alloys containing aluminum, and particularly aluminum-magnesium alloys, the valuable properties of the material, for example the limit of elongation, elasticity, hardness and 70 strength are very materially increased beyond anything obtainable by mechanical treatment.

If the final shape has not been given to the 75 material before subjecting it to my process, it may, for the purpose of obtaining definite qualities be submitted to cold treatment, as, for example, by rolling, drawing, pressing and like operations, which operations will have an effect on the qualities of the improved 80 material corresponding to that which such operations have on the qualities of metals usually subjected to such operations, viz: The limit of stretching, the strength and hardness are changed in a well known manner at the cost of elongation.

It is to be noted that any working of the 85 material directly after the heating to a high temperature and before storing it, impairs the result. Immaterial changes of shape, 90 however, are permissible, and this is of importance because many changes of shape, for example, straightening sheets of such metal, the production of sharp bends and flanging, cannot well be performed after the 95 storing.

The presence of magnesium in the alloy is important for obtaining the desired result. When the alloy also contains other metals, 100 for example, copper, manganese, nickel, titanium and the like, the advantages of my treatment are still further marked by a considerable additional increase in strength.

105 It has been found that the spontaneous improvement of the material after heating and during the storing, continues with the time of such storing, and this is particularly true in regard to the hardness.

110 It may be said that experience has shown that the hardness increases continually

through an infinite time interval, but the rate of increase of hardness is more rapid at first than later.

A measurable effect in the improvement 5 has been noticed after only about one and one half hours, and after twenty-four hours' storing a very decided improvement is found. In practice, it is advantageous to store for a longer time than twenty-four 10 hours because this results in a nearer approach to uniformity of the material, which, of course, is a considerable advantage. For this reason, in practice, it is well to store the material for about four days, although of 15 course, a shorter time may be sufficient.

For the purpose of illustrating the characteristic results which are attained by the improved process, it may be said that by heating to 500° C. and then chilling in water 20 plates made up of 99.5 per cent. aluminum and 0.5 per cent. magnesium, and then permitting the treated plates to rest for four days, without subjecting them to any further treatment or any substantial working 25 within that period, the hardness and tensile strength were approximately doubled as compared with pure aluminum.

Having thus fully described my invention, what I claim, is:—

1. The process of improving alloys containing aluminum and magnesium, which comprises heating the alloy to a temperature in excess of 420° C., thereafter cooling the alloy and allowing it to stand to permit spontaneous improvement. 35

2. The process of improving alloys containing aluminum and magnesium, which comprises working the alloy, then heating it to a temperature in excess of 420° C., slightly changing the shape of the alloy and 40 thereupon storing the alloy.

3. The process of improving alloys containing aluminum and magnesium, which comprises heating the alloy to a temperature between 420° C. and 580° C., thereafter 45 cooling the alloy and allowing it to stand to permit spontaneous improvement.

In testimony whereof, I affix my signature in the presence of two witnesses.

ALFRED WILM.

Witnesses:

WOLDEMAR HAUPT,  
HENRY HASPER.